

# UNITED STATES PATENT OFFICE.

FERNANDO SOMOZA VIVAS, OF SAN FRANCISCO, CALIFORNIA, ASSIGNOR OF ONE-HALF TO THEODORE A. BELL, OF SAN FRANCISCO, CALIFORNIA.

## VARNISH.

1,369,858.

Specification of Letters Patent. Patented Mar. 1, 1921.

No Drawing.

Application filed August 10, 1920. Serial No. 402,653.

To all whom it may concern:

Be it known that I, FERNANDO SOMOZA VIVAS, citizen of the United States, residing at San Francisco, in the county of San Francisco, and State of California, have invented certain new and useful Improvements in Varnishes, of which the following is a specification.

My invention relates to a fire-proofing varnish or coating, and it has for its object the provision of a material of this character which when applied to the surfaces of substances which are ordinarily destructible by fire will render the same in-

15 combustible.

A further object of my invention is the provision of a varnish or coating which will be highly weather-resisting, thus preserving the surfaces to which it is applied

20 from the deleterious action of the elements.

A further object of my invention is the making of a fire-proofing varnish or coating which shall be comparatively economical in cost of production and at the same 25 time highly efficient for the purpose for which it is designed.

To the above ends my invention consists in a varnish or surface coating composition composed of the following enumerated in-

gredients combined substantially in the proportions hereinafter set forth:

|                 |              |
|-----------------|--------------|
| Linseed oil     | 25 per cent. |
| Water           | 25 per cent. |
| Silver litharge | 25 per cent. |
| Sugar of lead   | 15 per cent. |
| A tungstate     | 5 per cent.  |
| Boric acid      | 5 per cent.  |

Having thus described my invention what I claim as new and desire to secure by Letters Patent is—

1. A fire-proofing varnish or coating composed of the following materials: linseed oil, water, silver litharge, sugar of lead, a tungstate and boric acid.

2. A fire-proofing varnish or coating composed of the following materials in substantially the relative proportions set forth: linseed oil 25 per cent., water 25 per cent., silver litharge 25 per cent., sugar of lead 15 per cent., a tungstate 5 per cent., and boric acid 5 per cent.

In testimony whereof I affix my signature in the presence of two witnesses.

FERNANDO SOMOZA VIVAS.

Witnesses:

F. MIRIAM MEYER,  
F. L. BROWNE.